

A. C. BIERNATZKI,  
SHEET FLOORING AND METHOD OF PRODUCING SAME,  
APPLICATION FILED JAN. 17, 1920.

1,382,595.

Patented June 21, 1921.



Inventor:  
*Albert C. Biernatzki*

By *Dodge and Dens*,  
Attorneys.

# UNITED STATES PATENT OFFICE.

ALBERT C. BIERNATZKI, OF AURORA, ILLINOIS.

## SHEET-FLOORING AND METHOD OF PRODUCING SAME.

1,382,595.

Specification of Letters Patent. Patented June 21, 1921.

Application filed January 17, 1920. Serial No. 352,053.

To all whom it may concern:

Be it known that I, ALBERT C. BIERNATZKI, a citizen of the United States, residing at Aurora, in the county of Kane and State 5 of Illinois, have invented certain new and useful Improvements in Sheet-Floorings and Methods of Producing Same, of which the following is a specification.

This invention pertains to an improved 10 flooring and to the method of producing the same. In certain portions of the middle west, and more particularly in the State of Utah, there is found a mineral known as asphalite which somewhat resembles in its 15 physical characteristics asphaltum, in that it may be reduced to a fluid condition by heat treatment and held in solution by suitable solvents such as naphtha and the like. There are several varieties of asphalite and 20 the most commonly known are those designated as elaterite and gilsonite, and these substances have been heretofore employed in the production of flooring surfaces, the former to a greater extent and more success- 25 fully than the latter. These materials when subjected to heat and held in solution by a suitable substance, such as naphtha, form a gummy substance or mastic. Elaterite or gilsonite thus held in solution have been 30 mixed with comminuted fibrous material and applied to the floor surface to be covered in successive layers, hydrated lime being sometimes mixed therewith to hasten the drying action. Where so laid successive 35 coatings have to be employed to insure the various coatings drying out and becoming sufficiently hard to withstand wear. Where it is attempted to apply the material in bulk of sufficient thickness to produce the 40 requisite floor covering, stair treads, desk tops, table tops, switch boards, and various other purposes of the kind where a hard smooth wearing surface is required, it is found that the material will not dry out 45 thoroughly except upon a long lapse of time. Where laid upon a wooden floor it will tend to check and to become otherwise defective by reason of the expansion and contraction of the wood. The great difficulty which 50 inheres in the use of this material produced from gilsonite or elaterite is that it dries very slowly and heretofore no way has been found, so far as I am aware, of producing the material in sheet form so that it may be 55 handled and shipped in sheet form substantially dry and ready for placement. The

present invention has to do with the production of the material in sheet form whereby it may be readily manufactured, transported and placed in position, the flooring 60 being substantially complete with the exception of the application of the finish coatings, which readily dry, though it is possible to produce a complete or finished sheet ready for direct laying by the user upon the floor. 65

One of the greatest difficulties which obtains in producing mastic in sheet form arises from the fact that it must be completed while it is in the plastic state, about the consistency of mortar, and the great adhesive property of the gum or mastic causes it to bond upon anything upon which it is spread for drying or while being rolled, making it impossible to take it up again so that it may be employed for any purpose. In 70 other words, up to the time of my invention it has been impossible, so far as I am aware, to pass the material between rollers while drying for the purpose of compression, getting a smooth surface, and by use of prop- 75 erly gaged rollers, obtaining an exact and uniform thickness of the sheet.

The material, according to the present invention, may be formed into sheets of the requisite size, and in the drawing I have 85 sought to show, in perspective, partly broken away, a portion of a sheet which is formed according to the method hereinafter set forth. I prefer to use elaterite rather than gilsonite owing to its superior inherent qual- 90 ities for the purposes in view.

In carrying out the invention, I employ a sheeting of fibrous material, preferably what is known as asbestos felt, which is designated in the drawing by 1. This sheet is partially 95 impregnated on the upper face with the mastic material above referred to, namely, the melted elaterite held in solution in a suitable solvent, such as naphtha, and imposed thereon is a layer of substantial thickness, 100 designated by 2, composed of the same material having distributed therethrough asbestos fiber or other fibrous material which tends to act as a binder and gives strength and wearing qualities to the ultimate struc- 105 ture, the elaterite giving tenacity, toughness, resiliency and elasticity. To produce this body, as 2, and the initial surface coating or layer, successive coatings of the mastic formed of elaterite in solution are ap- 110 plied and rolled, the rolling condensing the material and rendering it hard. The suc-

cessive coatings are permitted to dry for a short period of time, (about an hour) whereby the upper surface thereof becomes hardened to such an extent that it will not adhere to the roller. The body, however, remains plastic to such an extent that it may be rolled to smoothness and uniform thickness, but such rolling must take place before the hardening action strikes through the body of the layer. The handling of the sheet is rendered possible by the underlay of asbestos felt where otherwise it could not be manipulated. The sheets thus treated may be cut up to any desired shape or size.

15 Two methods have been employed to carry out this coating or building-up process. In one I employ wooden forms in which is laid asbestos felt and upon which the mastic is spread and rolled. Another 20 method is to place the felt upon a smooth floor surface, such as concrete, applying the mastic, then cutting it up, which may be done shortly after the application of the mastic to the felt, then running the material 25 between rollers to bring about the proper degree of compression and consequently density.

The material thus produced can be given any required degree of seasoning before being used. It may be piled or stacked without danger of the sheets adhering, this by reason of the employment of the felt sheet, inasmuch as the exposed face of the felt is not treated up to this time with the mastic.

30 The imposing of the successive layers of the mastic upon the felt does not sufficiently impregnate the exposed face thereof to such an extent that it will become sticky or tacky and thus adherence is prevented. When 35 laid, however, the exposed face of the felt is thoroughly saturated with the mastic which may be thinned out or partly dissolved so that it becomes, in effect, a paint which may be spread, and consequently the 40 felt body or sheet becomes impregnated and to all intents and purposes is practically the same as the body of the sheet. In other words, it becomes merely a mixture of asbestos and the mineral gum and will adhere 45 to wood, iron, or any dry surface.

50 In laying the floor composed of the sheets, the sheets are matched and cemented together with the use of the same mastic so that the joints do not show. The work can 55 be very much more rapidly done than with the use of mastic alone applied in successive coatings to the floors and the odor which is necessarily present when the material is applied in the manner just stated, is absent 60 to a very considerable degree, and consequently the floor may be laid and used where otherwise its employment would be barred.

The asbestos felt is also advantageous in that by its employment a seasoning of the 65 sheets of material may be governed. Sea-

soning, of course, is dependent upon exposure to the atmosphere. If the sheets are piled one upon another then naturally the seasoning is slow and they may be kept for a long period of time in a partially seasoned 70 condition. If fully exposed the material becomes as hard as a board and can not be readily applied. This feature is of material importance for the reason that if the sheets are not fully seasoned the application there- 75 of may be readily effected as they may be easily cut and fitted or may be bent to fit into a cove or corner or even wrapped about a pillar. Where it is sought to separate the sheets by the use of oil paper or the like, it 80 is found that the paper is apt to stick to the sheets and, what is more, the presence of the oil or grease is detrimental to the mastic as they tend to prevent proper adherence between the upper surface of the sheets when 85 laid and the finish coating 3 which may be applied thereto.

As above noted the sheeting may be formed complete prior to placement, or, if desired, a finish coating, as just noted, may 90 be applied. Preferably the sheets will be made up in three layers applied in separate 95 coatings, the first containing a large percentage of gum and a relatively small amount of asbestos, producing elasticity and acting as a cushion; the second formed of the same materials but containing a larger percentage of asbestos, which gives hardness and wearing qualities; and the third containing about the same percentage of gum 10 and asbestos as the second coating and in addition thereto the pigment or coloring matter which may be employed if desired.

In the claims I employ the term mineral 10 mastic as indicating a mass made up in the manner above set forth and produced either from the minerals elaterite or gilsonite (uintahite), though, as before indicated, I prefer to use elaterite owing to its superior qualities when employed for the purposes in 1 view.

It is, of course, conceivable that where a light flooring is to be employed but a single coating need be applied to the felt base, which coating when partially dry may be 1 passed through rolls to condense and gage the same as is done with the successively applied coatings where a heavier flooring is being produced.

What is claimed is:

1. As a new article of manufacture, sheet flooring comprising a fibrous base having a wearing body or tread surface of material thickness formed of mineral mastic as described imposed upon the base.
2. As a new article of manufacture, sheet flooring comprising a base of felt having a body of mineral mastic as described imposed and condensed thereon.
3. As a new article of manufacture, sheet

- flooring comprising a base of asbestos felt having a coating of paint produced from elaterite upon its exposed face and a body of mineral mastic imposed upon its opposite 5 face.
4. As a new article of manufacture, sheet flooring comprising a base of asbestos felt and a body formed from dissolved elaterite imposed thereon.
- 10 5. As a new article of manufacture, sheet flooring comprising a base of asbestos felt and a body of mineral mastic imposed thereon and having asbestos fiber intermixed therewith.
- 15 6. As a new article of manufacture sheet flooring comprising a base of asbestos felt and a body of mastic formed from elaterite having asbestos fiber intermixed therewith.
7. As a new article of manufacture, sheet 20 flooring comprising a base of asbestos felt; a body of mastic formed from elaterite having asbestos fiber intermixed therewith and a finish surface formed of elaterite mastic.
8. That method of producing sheet floor- 25 ing and maintaining the same in a more or less flexible condition ready for use, which consists in producing the sheets by imposing successive layers of mineral mastic upon a
- felt base to produce a body of material thickness; and piling the sheets thus produced to retard the hardening of the mastic.
9. That method of producing sheet flooring which consists in placing a sheet of asbestos felt upon a supporting surface; applying successive layers of mineral mastic there- 35 to; and condensing each layer prior to the placement of the next succeeding layer.
10. That method of producing sheet flooring which consists in placing a sheet of asbestos felt upon a supporting surface; ap- 40 plying thereto successive layers of mastic formed from elaterite; and condensing each layer prior to placement of the next succeed- 45 ing layer.
11. That method of producing sheet floor- ing which consists in placing a sheet of asbestos felt upon a supporting surface; applying thereto successive layers of mastic formed from elaterite having asbestos fibers inter- 50 mixed therewith; and condensing each layer prior to placement of the next succeeding layer.

In testimony whereof I have signed my name to this specification.

ALBERT C. BIERNATZKI.